

## UNITED STATES PATENT OFFICE

2,225,289

## PRINTING INK EXTENDER MANUFACTURE

William H. Wood, Bedford, Ohio, assignor to  
Harris-Seybold-Potter Company, Cleveland,  
Ohio, a corporation of Delaware

No Drawing. Application January 19, 1939,  
Serial No. 251,794

20 Claims. (Cl. 134—35)

It is common practice in printing, and especially lithographic printing, when a light tint of a particular color is desired, to dilute an ink of full color intensity with a white or colorless material so that the original pigment is extended throughout a larger volume of ink and the resulting tint of the print is accordingly lightened. When applying a white diluent or extender any desired tint from that of the original ink to white may be obtained. It is desirable however that the diluent be somewhat translucent, for the reason that a smaller proportion of the pigment, which is more costly than the diluent, would then be required in order to produce a given tint than if the diluent were opaque. Commonly, aluminum hydroxide is employed in linseed oil varnish as a diluent, and especially the commercial product known as "laketine," different samples of which have been found to vary widely in composition, being made up of varying amounts of aluminum hydroxide, zinc oxide, magnesium carbonate, linseed oil varnish, from one to twenty per cent of soap, and from two to thirty per cent of water. Such diluents have certain undesirable characteristics which render their use unsatisfactory, and particularly in lithographic printing. For example, they contain substances which react with the acids commonly used in lithographic plate dampening solutions to form compounds which are receptive to water. Such compounds attract water to the ink and cause emulsification thereof with harmful results, such as loss of intensity of color, "heavy front-end print," that is a heavier deposit of ink by the form rollers during their first revolution over the plate than during their second revolution, and a further particular difficulty is the serious scumming on the plate. These harmful results are enhanced by the water contents usual in the ink preparations. The water receptive compounds mentioned above furthermore tend to adhere to or react with the iron or metal rollers of the inker to form water-receptive areas on these rollers giving rise to "stripping" or removal of the ink from these areas. The commercial preparations as above mentioned, furthermore dry to a more or less greasy surface, thus making difficult the printing of a second color on previously printed areas, and also permitting too easy abrasion of a printed surface.

In accordance with the present invention it now becomes possible to avoid these well known drawbacks of the customary practice, and improved means for diluting or extending of printing inks or improvement of such diluents may be

had, and much more efficient operation of lithographic printing presses and the attainment of improved printed products.

To the accomplishment of the foregoing and related ends, the invention, then, comprises the features hereinafter fully described, and particularly pointed out in the claims, the following description setting forth in detail certain illustrative embodiments of the invention, these being indicative however, of but a few of the various ways in which the principle of the invention may be employed.

I have found that with suitable treatment a compound may be prepared based on the element zirconium, namely, the hydrous oxide of zirconium, to make an outstandingly successful extender for printing inks, and especially those for lithographic printing. It is micro-porous and therefore mixes particularly intimately with the other constituents of the ink. It, unlike many pigments, is colloidal in character, dispersing readily and not tending to separate out. It is substantially inert insofar as other constituents of printing inks are concerned. It does not react with the acids used in lithographic dampening solutions and thereby preserves the water-repellent character of the ink. It is blue-white in color and quite translucent, which characteristics make it particularly effective where highly diluted colors are desired. It is relatively inexpensive, and owing to its superior characteristics a relatively small quantity of pigment is required to produce a desired result. The materials in accordance with this invention furthermore provide a diluted ink which dries with a hard non-greasy surface particularly well adapted for receiving additional printings and not subject to easy abrasion. I have also found that in the same way I can employ certain other compounds, notably of titanium, and of silicon. In fact, under suitable conditions I can employ compounds of elements of the fourth group of the periodic system whose atomic number is at least 14, and in certain aspects the invention comprises such. It will be understood however that these compounds are not equivalents in all of the respects contemplated, but while the compound of zirconium is preferred, the grouping of zirconium and titanium is to be considered as available for some uses, and a grouping involving zirconium, titanium and silicon is available for certain uses, and compounds of the fourth periodic group generally of atomic number at least 14 are included for certain purposes. The compound prepared and em-

ployed in accordance with the invention is a colloidal material which is a hydrous oxide. In addition to the water which is bound in the molecule there is also unbound water normally present in a compound of this character owing to its hydrophilic nature. In preparation I largely remove the unbound water and retain the bound water and maintain the essential character of a hydrous oxide. One way of accomplishing this is by intimately mixing the material with a water-repellent vehicle, the mixing being carried on under conditions and for such time as suitable for the elimination of the unbound water desired. While various vehicles of such character may be employed, I prefer an oily vehicle of drying-oil type, and for instance particularly linseed oil varnish as of suitable drying characteristics for the printing ink industry.

As an example: Moist zirconium hydrous oxide, which may be manufactured by any desired method or preferably by precipitating from a water solution of a zirconium salt (for example the chloride or sulphate) by addition of ammonium hydroxide at ordinary temperature and filtering and washing, is introduced into an ink grinding mill together with linseed oil varnish of consistency suitable for ink usage. Grinding is continued until the unbound water is gradually eliminated and a uniform mixture of the zirconium compound and varnish is obtained. Grinding may be carried out on heated rolls or in a vacuum or both. Drying of the oxide by heat before grinding is not desirable for the reason that the translucent bulky hydrous oxide might thereby be converted over into the opaque dense ordinary oxide, thus losing the desired qualities of the hydrous oxide. The silicon compound also is precipitated by non-acid means. It will be observed that in any of the compounds contemplated in the usage of the present invention, an outstanding characteristic is the hydrous nature or hydrous oxide, the water content being well over half, altogether in contrast to the common oxides or hydroxides well known of the elements above-named. And by the term "hydrous oxide" in the specification and claims, I mean the voluminous gelatinous precipitate formed by reacting a hydroxide with a solution of a salt as indicated, such precipitate containing accessory elements of water in very large proportion of the whole and suitably separable as water.

In some cases I prefer to employ more than one of the hydrous oxides mentioned, these in mixture being incorporated conveniently together.

Other modes of applying the principle of the invention may be employed, change being made as regards the details described, provided the features stated in any of the following claims, or the equivalent of such, be employed.

I therefore particularly point out and distinctly claim as my invention:

1. As a new article of manufacture, a translucent extender for printing ink including as an essential constituent a colloidal agent which is a hydrous oxide of an element of the fourth group of the periodic table of atomic number at least 14 retaining its bound water and being chemically uncombined with other constituents.

2. As a new article of manufacture, a translucent extender for printing ink, comprising at least one compound from the group consisting of the hydrous oxides of zirconium, titanium, and silicon retaining its bound water, in a vehicle.

3. As a new article of manufacture, an extender

for printing ink, comprising zirconium hydrous oxide in a vehicle.

4. As a new article of manufacture, a translucent extender for printing ink, comprising titanium hydrous oxide in a vehicle.

5. As a new article of manufacture, a translucent extender for printing ink, comprising silicon hydrous oxide in a vehicle.

6. As a new article of manufacture, an extender for printing ink, comprising zirconium hydrous oxide in a drying vehicle.

7. As a new article of manufacture, an extender for printing ink, comprising zirconium hydrous oxide in a linseed oil vehicle.

8. As a new article of manufacture, a printing ink containing as an essential ingredient a translucent extender of colloidal hydrous oxide of an element of the fourth group of the periodic table of atomic number at least 14 retaining its bound water and being chemically uncombined with other constituents.

9. As a new article of manufacture, a printing ink containing as an essential ingredient a translucent extender of colloidal hydrous oxide of an element from the group consisting of zirconium, titanium and silicon retaining its bound water.

10. As a new article of manufacture, a printing ink containing zirconium hydrous oxide.

11. As a new article of manufacture, a printing ink containing a translucent extender of titanium hydrous oxide.

12. As a new article of manufacture, a printing ink containing a translucent extender of silicon hydrous oxide.

13. As a new article of manufacture, a printing ink containing zirconium hydrous oxide in a drying vehicle.

14. As a new article of manufacture, a printing ink containing zirconium hydrous oxide in a linseed oil vehicle.

15. In preparing lithographic printing ink, precipitating a hydrous oxide of one of the elements of the group consisting of zirconium, titanium and silicon from a water solution of a soluble salt by ammonium hydroxide, filtering and washing the precipitate, and grinding the precipitate while still moist in the presence of a drying oil vehicle until the unbound water is substantially eliminated.

16. In preparing lithographic printing ink, precipitating a hydrous oxide of zirconium from a water solution of a soluble zirconium salt by addition of ammonium hydroxide, filtering and washing the precipitate, and grinding the precipitate while still moist in the presence of a drying oil vehicle until the unbound water is substantially eliminated.

17. In the making of lithographic printing ink preparations, providing a moist hydrous oxide of an element of the fourth group of the periodic system having atomic weight at least 14, and before drying is permitted, grinding the moist hydrous material in substantial amount in a water-repellent vehicle until the unbound water is substantially eliminated and a translucent mixture is obtained.

18. In the making of lithographic printing ink preparations, providing a hydrous oxide of the group consisting of zirconium, titanium and silicon and containing unbound water, and before drying is permitted, grinding the moist hydrous material in substantial amount in a water-repellent vehicle until the unbound water is substantially eliminated and a translucent mixture is obtained.

19. In the making of lithographic printing ink preparations, providing a hydrous oxide of the group consisting of zirconium, titanium and silicon and containing unbound water, and before drying is permitted, grinding the moist hydrous material in substantial amount in a linseed oil varnish until the unbound water is substantially eliminated and a translucent mixture is obtained.
- 5 20. In the making of lithographic printing ink preparations, providing a hydrous oxide of zirconium, and before drying is permitted, grinding the moist hydrous material in substantial amount in a drying vehicle until the unbound water is 5 substantially eliminated.

WILLIAM H. WOOD.